



US005398153A

**United States Patent** [19]

Clough et al.

[11] Patent Number: **5,398,153**[45] Date of Patent: **Mar. 14, 1995**[54] **ELECTROSTATIC DISSIPATION AND ELECTROMAGNETIC INTERFERENCE SHIELDING ELEMENTS**[75] Inventors: **Thomas J. Clough, Santa Monica; Victor L. Grosvenor, Topanga; Naum Pinsky, Thousand Oaks, all of Calif.**[73] Assignee: **Ensci, Inc., Pismo Beach, Calif.**[21] Appl. No.: **714,598**[22] Filed: **Jun. 13, 1991****Related U.S. Application Data**

[60] Continuation-in-part of Ser. No. 348,787, May 8, 1989, abandoned, which is a continuation-in-part of Ser. No. 272,517, Nov. 17, 1988, abandoned, and a continuation-in-part of Ser. No. 272,539, Nov. 17, 1988, abandoned, each is a continuation-in-part of Ser. No. 82,277, Aug. 6, 1987, Pat. No. 4,787,125, which is a division of Ser. No. 843,047, Mar. 24, 1986, Pat. No. 4,713,306.

[51] Int. Cl.<sup>6</sup> ..... **H05F 3/00**[52] U.S. Cl. ..... **361/212**[58] Field of Search ..... **252/518; 361/212; 523/137**[56] **References Cited****U.S. PATENT DOCUMENTS**

|           |         |                    |         |
|-----------|---------|--------------------|---------|
| 3,005,731 | 10/1961 | Payne              | 117/211 |
| 3,544,361 | 6/1966  | Servais            | 117/124 |
| 3,562,124 | 2/1971  | Leon et al.        | 204/148 |
| 3,562,127 | 2/1971  | Wooton et al.      | 204/164 |
| 3,713,884 | 1/1973  | Maley              | 117/211 |
| 3,870,567 | 3/1975  | Palmer et al.      | 136/148 |
| 3,890,429 | 6/1975  | Ptylewski          | 423/395 |
| 3,959,565 | 5/1976  | Jordan et al.      | 428/432 |
| 4,229,491 | 10/1980 | Dislich et al.     | 427/160 |
| 4,258,080 | 3/1981  | Sonoda et al.      | 427/82  |
| 4,275,130 | 1/1981  | Rippel et al.      | 429/144 |
| 4,297,420 | 10/1981 | Chenaux et al.     | 429/217 |
| 4,349,369 | 9/1982  | Van Laethem et al. | 65/60.4 |
| 4,371,740 | 2/1983  | Clem               | 136/256 |
| 4,405,697 | 9/1983  | Rowlette           | 429/161 |
| 4,510,219 | 4/1985  | Rowlette           | 429/212 |
| 4,517,118 | 5/1985  | Stoetzer           | 252/513 |

|           |         |                  |           |
|-----------|---------|------------------|-----------|
| 4,535,315 | 8/1985  | Sakai            | 338/34    |
| 4,539,268 | 9/1985  | Rowlette         | 429/54    |
| 4,542,082 | 9/1985  | Rowlette         | 429/210   |
| 4,547,443 | 10/1985 | Rowlette et al.  | 429/217   |
| 4,818,437 | 4/1989  | Wiley            | 252/511   |
| 4,818,438 | 4/1989  | Wiley            | 252/511   |
| 4,889,750 | 12/1989 | Wiley            | 428/34.2  |
| 5,204,140 | 4/1993  | Grosvenor et al. | 427/126.3 |

**FOREIGN PATENT DOCUMENTS**

|         |        |                    |
|---------|--------|--------------------|
| 0116785 | 8/1984 | European Pat. Off. |
| 0130575 | 1/1985 | European Pat. Off. |

**OTHER PUBLICATIONS**

"Electroless Deposition of SnO<sub>2</sub> and Antimony Doped SnO<sub>2</sub> Films", D. Raviendra et al, J. Phys Chem Solids vol. 46 No. 8, pp. 945-950, 1985 USA.  
 "Sn(Sb)-Oxide Sol-Gel Coatings on Glass", C. J. R. Gonzalez-Oliver et al, J Non-Crystalline Solids 82, pp. 400-410, 1986, Amsterdam.  
 "Physical Properties of Tin Oxide Films Deposited By Oxidation of SnCl<sub>2</sub>", N. S. Murty et al, Thin Solid Films 92, pp. 347-354 1982 The Netherlands.

(List continued on next page.)

*Primary Examiner*—Jeffrey A. Gaffin  
*Attorney, Agent, or Firm*—Frank J. Uxa, Jr.

[57] **ABSTRACT**

An electrostatic dissipation/electromagnetic interference shielding element comprising a three dimensional substrate having shielded surfaces which are at least partially shielded by other portions of said substrate and having an electronically conductive tin oxide-containing coating on at least a portion of all three dimensions thereof and said shielded surface, said coated substrate being adapted and structured to provide at least one of the following: electrostatic dissipation and electromagnetic interference shielding.

**31 Claims, 2 Drawing Sheets**

OTHER PUBLICATIONS

"Tin Dioxide Gas Sensors", Part 1, J. F. McAleer et al. J Chem Soc, Faraday Trans I, 83, pp. 1323-1346, 1987.  
"Tin Dioxide Gas Sensors", Part 2, J. F. McAleer et al, J. Chem Soc. Faraday Trans I, 84, pp. 441-457, 1988.  
"Preparation of Thick Crystalline Films of Tin Oxide and Porous Glass Partially Filled with Tin Oxide", Bartholomew et al., J. Electrochem Soc, 116, pp. 1205-1208, 1969.  
"The Catalyzed Conversion of Methane to Methanol at

High Pressure", N. R. Hunter et al, Symp Hydrocarbon Oxidation, Amer Chem Soc. 1987.  
"Compression Molding of Conductive Plastics", D. E. Davenport.  
"Sol-Gel AR Films for Solar Applications", C. S. Ashley et al, work performed at Sandia National Laboratories.  
"Sol-Gel Glass Research", Technology Forecasts and Technology Surveys, pp. 5-7, 1983.  
"Tin Oxide Films on Glass Substrates by a Sol-Gel Technique", R. Puyane et al, pp. 190-197.



Fig. 1



**ELECTROSTATIC DISSIPATION AND  
ELECTROMAGNETIC INTERFERENCE  
SHIELDING ELEMENTS**

**RELATED APPLICATIONS**

This application is a continuation-in-part of application Ser. No. 348,787, now abandoned, filed May 8, 1989, which is a continuation-in-part of application Ser. Nos. 272,517, now abandoned and 272,539, now abandoned each filed Nov. 17, 1988, each of which applications is a continuation-in-part of application Ser. No. 082,277, filed Aug. 6, 1987, now U.S. Pat. No. 4,787,125 which application, in turn, is a division of application Ser. No. 843,047, filed Mar. 24, 1986, now U.S. Pat. No. 4,713,306. These earlier filed applications and these U.S. Patents are incorporated in their entireties herein by reference.

**BACKGROUND OF THE INVENTION**

The present invention relates to a new electrostatic dissipation/electromagnetic interference shielding element. More particularly, the invention relates to an element having an inorganic substrate with a tin oxide-containing material, preferably an electronically conductive tin oxide-containing material.

In the above-noted applications it would be advantageous to have an electronically conductive tin oxide which is substantially uniform, has high electronic conductivity, and has good chemical properties, e.g., morphology, stability, etc.

A number of techniques may be employed to provide conductive tin oxide coatings on acid resistant substrates. For example, the chemical vapor deposition (CVD) process may be employed. This process comprises contacting a substrate with a vaporous composition comprising a tin component and a dopant-containing material and contacting the contacted substrate with an oxygen-containing vaporous medium at conditions effective to form the doped tin oxide coating on the substrate. Conventionally, the CVD process occurs simultaneously at high temperatures at very short contact times so that tin oxide is initially deposited on the substrate. However tin oxide can form off the substrate resulting in a low reagent capture rate. The CVD process is well known in the art for coating a single flat surface which is maintained in a fixed position during the above-noted contacting steps. The conventional CVD process is an example of a "line-of-sight" process or a "two dimensional" process in which the tin oxide is formed only on that portion of the substrate directly in the path of the tin source as tin oxide is formed on the substrate. Portions of the substrate which are shielded from the tin oxide being formed, e.g., such as pores which extend inwardly from the external surface and substrate layers which are at least partially shielded from the depositing tin oxide by one or more other layers closer to the external substrate surface, do not get uniformly coated, if at all, in a "line-of-sight" process. A particular problem with "line-of-sight" processes is the need to maintain a fixed distance between the tin source and the substrate. Otherwise, tin dioxide can be deposited or formed off the substrate and lost, with a corresponding loss in process and reagent efficiency.

Although the CVD process is useful for coating a single flat surface, for the reasons noted above this process tends to produce non-uniform and/or discontinuous coatings on woven glass fiber mats. Such non uni-

formities and/or discontinuities are detrimental to the electrical and chemical properties of the coated substrate. A new process, e.g., a "non-line-of-sight" or "three dimensional" process, useful for coating such substrates would be advantageous. As used herein, a "non-line-of-sight" or "three dimensional" process is a process which coats surfaces of a substrate with tin oxide which surfaces would not be directly exposed to vaporous tin oxide-forming compounds being deposited on the external surface of the substrate during the first contacting step. In other words, a "three dimensional" process coats coatable substrate surfaces which are at least partially shielded by other portions of the substrate which are closer to the external surface of the substrate, e.g., the surfaces of the internal fibers of a porous mat of glass fibers.

Although a substantial amount of work has been done, there continues to be a need for a new method for coating substrates with doped tin oxide.

**SUMMARY OF THE INVENTION**

A new electrostatic dissipation/electromagnetic interference shielding element has been discovered particularly a three dimensional inorganic substrate having an electronically doped conductive tin oxide containing coating on at least a portion of all three dimensions thereof, said coated substrate being adapted and structured to provide at least one of the following: electrostatic dissipation and electromagnetic interference shielding. A very useful application of this invention is for static, for example electrostatic dissipation and shielding particularly for ceramic and polymeric parts having the tin oxide coated inorganic substrates incorporated therein. The tin oxide coated substrates for use in the products of this invention can be made by a process for coating at least a portion of all three dimensions of said substrate including at least a portion of the shielded surfaces of said substrates. The process comprises contacting the substrate with stannous chloride, in a vaporous form and/or in a liquid form, to form a stannous chloride-containing coating on the substrate; contacting the substrate with a fluorine component, i.e., a component containing free fluorine and/or combined fluorine (as in a compound), to form a fluorine component-containing coating on the substrate; and contacting the thus coated substrate with an oxidizing agent to form a fluorine doped tin oxide, preferably tin dioxide, coating on the substrate. The contacting of the substrate with the stannous chloride and with the fluorine component can occur together, i.e., simultaneously, and/or in separate steps.

Substantial coating uniformity, e.g., in the thickness of the tin oxide-containing coating and in the distribution of dopant component in the coating, is obtained. Further, the present fluorine doped tin oxide coated substrates have outstanding stability, e.g., in terms of electrical properties and morphology, and are thus useful in various applications. In addition, the process is efficient in utilizing the materials which are employed to form the coated substrate.

**DETAILED DESCRIPTION OF THE  
INVENTION**

In one broad aspect, the present coating process comprises contacting a substrate with a composition comprising a tin oxide precursor, such as tin chloride forming components, including stannic chloride, stannous

chloride and mixtures thereof, preferably stannous chloride, at conditions, preferably substantially non-deleterious oxidizing conditions, more preferably in a substantially inert environment or atmosphere, effective to form a tin oxide precursor-containing coating, such as a stannous chloride-containing coating, on at least a portion of the substrate. The substrate is preferably also contacted with at least one dopant-forming component, such as at least one fluorine component, at conditions, preferably substantially non-deleterious oxidizing conditions, more preferably in a substantially inert atmosphere, effective to form a dopant-forming component-containing coating, such as a fluorine component-containing coating, on at least a portion of the substrate. This substrate, including one or more coatings containing tin oxide precursor, for example tin chloride and preferably stannous chloride, and preferably a dopant-forming component, for example a fluorine component, is contacted with at least one oxidizing agent at conditions effective to convert the tin oxide precursor to tin oxide and form a tin oxide-containing, preferably tin dioxide-containing, coating, preferably a doped, e.g., fluorine or fluoride doped, tin oxide-containing coating, on at least a portion of the substrate. By "non-deleterious oxidation" is meant that the majority of the oxidation of tin oxide precursor, for example stannous chloride, coated onto the substrate takes place in the oxidizing agent contacting step of the process, rather than in process step or steps conducted at non-deleterious oxidizing conditions. The process as set forth below will be described in many instances with reference to stannous chloride, which has been found to provide particularly outstanding process and product properties. However, it is to be understood that other suitable tin oxide precursors are included within the scope of the present invention.

The dopant-forming component-containing coating may be applied to the substrate before and/or after and/or during the time the substrate is coated with stannous chloride. In a particularly useful embodiment, the stannous chloride and the dopant-forming component are both present in the same composition used to contact the substrate so that the stannous chloride-containing coating further contains the dopant-forming component. This embodiment provides processing efficiencies since the number of process steps is reduced (relative to separately coating the substrate with stannous chloride and dopant-forming component). In addition, the relative amount of stannous chloride and dopant-forming component used to coat the substrate can be effectively controlled in this "single coating composition" embodiment of the present invention.

In another useful embodiment, the substrate with the stannous chloride-containing coating and the dopant-forming component-containing coating is maintained at conditions, preferably at substantially non-deleterious oxidizing conditions, for a period of time effective to do at least one of the following: (1) coat a larger portion of the substrate with stannous chloride-containing coating; (2) distribute the stannous chloride coating over the substrate; (3) make the stannous chloride-containing coating more uniform in thickness; and (4) distribute the dopant-forming component more uniformly in the stannous chloride-containing coating. Such maintaining preferably occurs for a period of time in the range of about 0.1 minute to about 20 minutes. Such maintaining is preferably conducted at the same or a higher temperature relative to the temperature at which the sub-

strate/stannous chloride-containing composition contacting occurs. Such maintaining, in general, acts to make the coating more uniform and, thereby, for example, provides for beneficial electrical conductivity properties. The thickness of the tin oxide-containing coating is preferably in the range of about 0.1 micron to about 10 microns, more preferably about 0.25 micron to about 1.25 microns.

The stannous chloride which is contacted with the substrate is in a vaporous phase or state, or in a liquid phase or state, or in a solid state or phase (powder) at the time of the contacting. The composition which includes the stannous chloride preferably also includes the dopant-forming component or components. This composition may also include one or more other materials, e.g., dopants, catalysts, grain growth inhibitors, solvents, etc., which do not substantially adversely promote the premature hydrolysis of the stannous chloride and/or the dopant-forming component, and do not substantially adversely affect the properties of the final product, such as by leaving a detrimental residue in the final product prior to the formation of the tin oxide-containing coating. Thus, it has been found to be important, e.g., to obtaining a tin oxide coating with good structural and/or electronic properties, that undue hydrolysis of the stannous chloride and dopant-forming component be avoided. This is contrary to certain of the prior art which actively utilized the simultaneous hydrolysis reaction as an approach to form the final coating. Examples of useful other materials include organic components such as acetonitrile, ethyl acetate, dimethyl sulfoxide, propylene carbonate and mixtures thereof; certain inorganic salts and mixtures thereof. These other materials, which are preferably substantially anhydrous, may often be considered as a carrier, e.g., solvent, for the stannous chloride and/or dopant-forming component to be contacted with the substrate. It has also been found that the substrate can first be contacted with a tin oxide precursor powder, particularly stannous chloride powder, preferably with a film forming amount of such powder, followed by increasing the temperature to the liquidus point of the powder on the substrate and maintaining the coated substrate for a period of time at conditions including the increased temperature effective to do at least one of the following: (1) coat a larger portion of the substrate with the tin oxide precursor-containing coating; (2) distribute the coating over the substrate; and (3) make the coating more uniform in thickness. Preferably, this step provides for the equilibration of the coating on the substrate. The size distribution of the powder, for example, stannous chloride powder, and the amount of such powder applied to the substrate are preferably chosen so as to distribute the coating over substantially the entire substrate.

Typical tin oxide precursor powders are those that are powders at powder/substrate contacting conditions and which are liquidus at the maintaining conditions, preferably equilibration conditions, of the present process.

In addition to the other materials, as noted above, the composition containing stannous chloride and/or the dopant-forming component may also include one or more grain growth inhibitor components. Such inhibitor component or components are present in an amount effective to inhibit grain growth in the tin oxide-containing coating. Reducing grain growth leads to beneficial coating properties, e.g., higher electrical conductivity, more uniform morphology, and/or greater overall

stability. Among useful grain growth inhibitor components are components which include at least one metal, in particular potassium, calcium, magnesium, silicon and mixtures thereof. Of course, such grain growth inhibitor components should have no substantial detrimental effect on the final product.

The dopant-forming component may be deposited on the substrate separately from the stannous chloride, e.g., before and/or during and/or after the stannous chloride/substrate contacting. If the dopant-forming component is deposited on the substrate separately from the stannous chloride, it is preferred that the dopant-forming component, for example, the fluorine component, be deposited after the stannous chloride.

Any suitable dopant-forming component may be employed in the present process. Such dopant-forming component should provide sufficient dopant so that the final doped tin oxide coating has the desired properties, e.g., electronic conductivity, stability, etc. Fluorine components are particularly useful dopant-forming components. Care should be exercised in choosing the dopant-forming component or components for use. For example, the dopant-forming component should be sufficiently compatible with the stannous chloride so that the desired doped tin oxide coating can be formed. Dopant-forming components which have excessively high boiling points and/or are excessively volatile (relative to stannous chloride), at the conditions employed in the present process, are to be avoided since, for example, the final coating may not be sufficiently doped and/or a relatively large amount of the dopant-forming component or components may be lost during processing. It may be useful to include one or more property altering components, e.g., boiling point depressants, in the composition containing the dopant-forming component to be contacted with the substrate. Such property altering component or components are included in an amount effective to alter one or more properties, e.g., boiling point, of the dopant-forming component, e.g., to improve the compatibility or reduce the incompatibility between the dopant-forming component and stannous chloride.

Particularly useful fluorine components for use in the present invention are selected from stannous fluoride, stannic fluoride, hydrogen fluoride and mixtures thereof. When stannous fluoride is used as a fluorine component, it is preferred to use one or more boiling point depressants to reduce the apparent boiling point of the stannous fluoride, in particular to at least about 850° C. or less.

The use of a fluorine or fluoride dopant is an important feature of certain aspects of the present invention. First, it has been found that fluorine dopants can be effectively and efficiently incorporated into the tin oxide-containing coating. In addition, such fluorine dopants act to provide tin oxide-containing coatings with good electronic properties referred to above, morphology and stability. This is in contrast to certain of the prior art which found antimony dopants to be ineffective to improve the electronic properties of tin oxide coatings in specific applications.

The substrate including the stannous chloride-containing coating and the dopant-forming component-containing coating is contacted with an oxidizing agent at conditions effective to convert stannous chloride to tin oxide, preferably substantially tin dioxide, and form a doped tin oxide coating on at least a portion of the substrate. Water, e.g., in the form of a controlled

amount of humidity, is preferably present during the coated substrate/oxidizing agent contacting. This is in contrast with certain prior tin oxide coating methods which are conducted under anhydrous conditions. The presence of water during this contacting has been found to provide a doped tin oxide coating having excellent electrical conductivity properties.

Any suitable oxidizing agent may be employed, provided that such agent functions as described herein. Preferably, the oxidizing agent (or mixtures of such agents) is substantially gaseous at the coated substrate/oxidizing agent contacting conditions. The oxidizing agent preferably includes reducible oxygen, i.e., oxygen which is reduced in oxidation state as a result of the coated substrate/oxidizing agent contacting. More preferably, the oxidizing agent comprises molecular oxygen, either alone or as a component of a gaseous mixture, e.g., air.

The substrate may be composed of any suitable material and may be in any suitable form. Preferably, the substrate is such so as to minimize or substantially eliminate the migration of ions and other species, if any, from the substrate to the tin oxide-containing coating which are deleterious to the functioning or performance of the coated substrate in a particular application. In addition, it can be precoated to minimize migration, for example a silica precoat and/or to improve wettability and uniform distribution of the coating materials on the substrate. In order to provide for controlled electronic conductivity in the doped tin oxide coating, it is preferred that the substrate be substantially non-electronically conductive when the coated substrate is to be used as a component of an electric energy storage battery. In one embodiment, the substrate is inorganic, for example glass and/or ceramic. Although the present process may be employed to coat two dimensional substrates, such as substantially flat surfaces, it has particular applicability in coating three dimensional substrates. Thus, the present process is a three dimensional process. Examples of three dimensional substrates which can be coated using the present process include spheres, extrudates, flakes, single fibers, fiber rovings, chopped fibers, fiber mats, porous substrates, irregularly shaped particles, e.g., catalyst supports, multi-channel monoliths and the like. Acid resistant glass fibers, especially woven and non-woven mats of acid resistant glass fibers, are particularly useful substrates when the doped tin oxide coated substrate is to be used as a component of a battery, such as a lead-acid electrical energy storage battery. More particularly, the substrate for use in a battery is in the form of a body of woven or non-woven fibers, still more particularly, a body of fibers having a porosity in the range of about 60% to about 95%. Porosity is defined as the percent or fraction of void space within a body of fibers. The above-noted porosities are calculated based on the fibers including the desired fluorine doped tin oxide coating. The substrate for use in lead-acid batteries, because of availability, cost and performance considerations, preferably comprises acid resistant glass, more preferably in the form of fibers, as noted above.

The tin oxide coated substrate, such as the fluorine doped tin oxide coated substrate, of the present invention may be, for example, a catalyst itself or a component of a composite together with one or more matrix materials. The composites may be such that the matrix material or materials substantially totally encapsulate or surround the coated substrate, or a portion of the coated

substrate may extend away from the matrix material or materials.

Any suitable matrix material or materials may be used in a composite with the tin oxide coated substrate. Preferably, the matrix material comprises a polymeric material, e.g., one or more synthetic polymers, more preferably an organic polymeric material. The polymeric material may be either a thermoplastic material or a thermoset material. Among the thermoplastics useful in the present invention are the polyolefins, such as polyethylene, polypropylene, polymethylpentene and mixtures thereof; and poly vinyl polymers, such as polystyrene, polyvinylidene difluoride, combinations of polyphenylene oxide and polystyrene, and mixtures thereof. Among the thermoset polymers useful in the present invention are epoxies, phenol-formaldehyde polymers, polyesters, polyvinyl esters, polyurethanes, melamine-formaldehyde polymers, and urea-formaldehyde polymers.

In order to provide enhanced bonding between the tin oxide coated substrate and the matrix material, it has been found that the preferred matrix materials have an increased polarity, as indicated by an increased dipole moment, relative to the polarity of polypropylene. Because of weight and strength considerations, if the matrix material is to be a thermoplastic polymer, it is preferred that the matrix be a polypropylene-based polymer which includes one or more groups effective to increase the polarity of the polymer relative to polypropylene. Additive or additional monomers, such as maleic anhydride, vinyl acetate, acrylic acid, and the like and mixtures thereof, may be included prior to propylene polymerization to give the product propylene-based polymer increased polarity. Hydroxyl groups may also be included in a limited amount, using conventional techniques, to increase the polarity of the final propylene-based polymer.

Thermoset polymers which have increased polarity relative to polypropylene are more preferred for use as the present matrix material. Particularly preferred thermoset polymers include epoxies, phenol-formaldehyde polymers, polyesters, and polyvinyl esters.

A more complete discussion of the presently useful matrix materials is presented in Fitzgerald, et al U.S. Pat. No. 4,708,918, the entire disclosure of which is hereby incorporated by reference herein.

Various techniques, such as casting, molding and the like, may be used to at least partially encapsulate or embed the tin oxide coated substrate into the matrix material or materials and form composites. The choice of technique may depend, for example, on the type of matrix material used, the type and form of the substrate used and the specific application involved. Certain of these techniques are presented in U.S. Pat. No. 4,547,443, the entire disclosure of which is hereby incorporated by reference herein. One particular embodiment involves pre-impregnating (or combining) that portion of the tin oxide coated substrate to be embedded in the matrix material with a relatively polar (increased polarity relative to polypropylene) thermoplastic polymer, such as polyvinylidene difluoride, prior to the coated substrate being embedded in the matrix material. This embodiment is particularly useful when the matrix material is itself a thermoplastic polymer, such as modified polypropylene, and has been found to provide improved bonding between the tin oxide coated substrate and the matrix material.

In order to provide for improved bonding of the fluorine doped tin oxide coating (on the substrate) with the matrix material, it is preferred to at least partially, more preferably substantially totally, coat the fluorine doped tin oxide coated substrate with a coupling agent which acts to improve the bonding of the fluorine doped tin oxide coating with the matrix. This is particularly useful when the substrate comprises acid resistant glass fibers. Any suitable coupling agent may be employed.

Such agents preferably comprise molecules which have both a polar portion and a non-polar portion. Certain materials generally in use as sizing for glass fibers may be used here as a "size" for the doped tin oxide coated glass fibers. The amount of coupling agent used to coat the fluorine doped tin oxide coated glass fibers should be effective to provide the improved bonding noted above and, preferably, is substantially the same as is used to size bare glass fibers. Preferably, the coupling agent is selected from the group consisting of silanes, silane derivatives, stannates, stannate derivatives, titanates, titanate derivatives and mixtures thereof. U.S. Pat. No. 4,154,638 discloses one silane-based coupling agent adapted for use with tin oxide surfaces. The entire disclosure of this patent is hereby expressly incorporated by reference herein.

The tin oxide/substrate combinations, e.g., the tin oxide coated substrates, of the present invention are useful in other applications as well. Among these other applications are included porous membranes, resistance heating elements, electrostatic dissipation elements, electromagnetic interference shielding elements, protective coatings and the like.

In one embodiment, a porous membrane is provided which comprises a porous substrate, preferably an inorganic substrate, and a tin oxide-containing material in contact with at least a portion of the porous substrate. In another embodiment, the porous membrane comprises a porous organic matrix material, e.g., a porous polymeric matrix material, and a tin oxide-containing material in contact with at least a portion of the porous organic matrix material. With the organic matrix material, the tin oxide-containing material may be present in the form of an inorganic substrate, porous or substantially non porous, having a tin oxide-containing coating, e.g., an electronically conductive tin oxide-containing coating, thereon.

One particularly useful feature of the present porous membranes is the ability to control the amount of tin oxide present to provide for enhanced performance in a specific application, e.g., a specific contacting process. For example, the thickness of the tin oxide-containing coating can be controlled to provide such enhanced performance. The coating process of the present invention is particularly advantageous in providing such controlled coating thickness. Also, the thickness of the tin oxide-containing coating can be varied, e.g., over different areas of the same porous membrane, such as an asymmetric porous membrane. In fact, the thickness of this coating can effect the size, e.g., diameter, of the pores. The size of the pores of the membrane or porous substrate may vary inversely with the thickness of the coating. The coating process of the present invention is particularly useful in providing this porosity control.

In one embodiment, a flexible heating element is provided which comprises a flexible matrix material, e.g., an organic polymeric material in contact with a substrate having an electronically conductive tin oxide-containing coating on at least a portion thereof. The

coated substrate is adapted and structured as described above.

In addition, an electrostatic dissipation/electromagnetic interference shielding element is provided which comprises a three dimensional substrate, e.g., an inorganic substrate, having an electronically conductive tin oxide-containing coating on at least  $2a$  portion of all three dimensions thereof. The coated substrate is adapted and structured to provide at least one of the following: electrostatic dissipation and electromagnetic interference shielding.

A very useful application for the products of this invention is for static, for example, electrostatic, dissipation and shielding, particularly for ceramic and polymeric parts, and more particularly as a means for effecting static dissipation including controlled static charge and dissipation such as used in certain electro static painting processes and/or electric field absorption in parts, such as parts made of ceramics and polymers and the like, as described herein. The present products can be incorporated directly into the polymer or ceramic and/or a carrier such as a cured or uncured polymer based carrier or other liquid, as for example in the form of a liquid, paste, hot melt, film and the like. These product/carrier based materials can be directly applied to parts to be treated to improve overall performance effectiveness. A heating cycle is generally used to provide for product bonding to the parts. A particular unexpected advantage is the improved mechanical properties, especially compared to metallic additives which may compromise mechanical properties. In addition, the products of this invention can be used in molding processes to allow for enhanced static dissipation and/or shielding properties of polymeric resins relative to an article or device or part without such product or products, and/or to have a preferential distribution of the product or products at the surface of the part for greater volume effectiveness within the part.

The particular form of the products, i.e., fibers, flakes, particles, mats or the like, is chosen based upon the particular requirements of the part and its application, with one or more of flakes, fibers and particles being preferred for polymeric parts. In general, it is preferred that the products of the invention have a largest dimension, for example, the length of fiber or side of a flake, of less than about  $\frac{1}{8}$  inch, more preferably less than about  $1/64$  inch and still more preferably less than about  $1/128$  inch. It is preferred that the ratio of the longest dimension, for example, length, side or diameter, to the shortest dimension of the products of the present invention be in the range of about 500 to 1 to about 10 to 1, more preferably about 250 to 1 to about 25 to 1. The concentration of such product or products in the product/carrier and/or mix is preferably less than about 60 weight %, more preferably less than about 40 weight %, and still more preferably less than about 20 weight %. A particularly useful concentration is that which provides the desired performance while minimizing the concentration of product in the final article, device or part.

The products of this invention find particular advantage in static dissipation parts, for example, parts having a surface resistivity in the range of about  $10^4$  ohms/square to about  $10^{12}$  ohms/square. In addition, those parts generally requiring shielding to a surface resistivity in the range of about 1 ohm/square to about  $10^5$  ohms/square and higher find a significant advantage for the above products due to their mechanical properties

and overall improved polymer compatibility, for example, matrix bonding properties as compared to difficult to bond metal and carbon-based materials. A further advantage of the above products is their ability to provide static dissipation and/or shielding in adverse environments such as in corrosive water and/or electro galvanic environments. As noted above, the products have the ability to absorb as well as to reflect electro fields. The unique ability of the products to absorb allows parts to be designed which can minimize the amount of reflected electro fields that is given off by the part. This latter property is particularly important where the reflected fields can adversely affect performance of the part.

A flexible electrostatic dissipation/electromagnetic interference shielding element is also included in the scope of the present invention. This flexible element comprises a flexible matrix material, e.g., an organic polymeric material, in contact with a substrate having an electronically conductive tin oxide-containing coating on at least a portion thereof. The coated substrate of this flexible element is adapted and structured as described above.

The present coating process is particularly suitable for controlling the composition and structure of the coating on the substrate to enhance the performance of the coated substrate in a given, specific application, e.g., a specific resistance heating electrostatic dissipation or electromagnetic interference shielding application.

Particular applications which combine many of the outstanding properties of the products of the present invention include porous and electro membrane separations for food processing, textile/leather processing, chemical processing, bio medical processing and water treatment. For example, various types of solutions can be further concentrated, e.g., latex concentrated, proteins isolated, colloids removed, salts removed, etc. The membranes can be used in flat plate, tubular and/or spiral wound system design. In addition, the products of this invention can be used e.g., as polymeric composites, for electromagnetic and electrostatic interference shielding applications used for computers, telecommunications and electronic assemblies, as well as in low radar observable systems and static dissipation, for example, in carpeting and in lightning protection systems for aircraft.

The porous membrane, in particular the substrate, can be predominately organic or inorganic, with an inorganic substrate being suitable for demanding process environments. The porous organic-containing membranes often include a porous organic based polymer matrix material having incorporated therein a three dimensional tin oxide-containing material, preferably including an electronically conductive tin dioxide coating, more preferably incorporating a dopant and/or a catalytic species, in an amount that provides the desired function, particularly electrical conductivity, without substantially deleteriously affecting the properties of the organic polymer matrix material. These modified polymer membranes are particularly useful in porous membrane and/or electromembrane and/or catalytic processes.

#### BRIEF DESCRIPTION OF THE DRAWINGS

FIG. 1 is a block flow diagram illustrating a process for producing the present coated substrates.

FIG. 2 is a schematic illustration showing an embodiment of the electromagnetic interference shielding element of the present invention in use.

FIG. 3 is a schematic illustration showing an embodiment of the electrostatic dissipation element of the present invention in use.

FIG. 4 is a detailed, somewhat schematic illustration of a portion of the electromagnetic interference shielding element shown in FIG. 2.

FIG. 5 is a blown-up, cross-sectional view of an individual coated fiber of the coated substrate shown in FIG. 4.

FIG. 6 is a detailed, somewhat schematic illustration of a portion of the electrostatic dissipation element shown in

#### DETAILED DESCRIPTION OF THE DRAWINGS

The following description specifically involves the coating of randomly oriented, woven mats of C-glass fibers. However, it should be noted that substantially the same process steps can be used to coat other substrate forms and/or materials.

A process system according to the present invention, shown generally at 10, includes a preheat section 12, a coating section 14, an equilibration section 16 and an oxidation/sintering section 18. Each of these sections is in fluid communication with the others. Preferably, each of these sections is a separate processing zone or section.

First gas curtain 20 and second gas curtain 22 provide inert gas, preferably nitrogen, at the points indicated, and, thereby effectively insure that preheat section 12, coating section 14 and equilibrium section 16 are maintained in a substantially inert environment. First exhaust 24 and second exhaust 26 are provided to allow vapors to exit or be vented from process system 10.

Randomly oriented woven mats of C-glass fibers from substrate source 28 are fed to preheat section 12 where the mats are preheated up to a maximum of 375° C. for a time of 1 to 3 minutes at atmospheric pressure to reach thermal equilibrium. These mats are composed of from 8 micron to 35 micron diameter C- or T-glass randomly oriented or woven fibers. The mats are up to 42 inches wide and between 0.058 to 0.174 mil thick. The mats are fed to process system 10 at the rate of about 1 to 5 feet per minute so that the fiber weight throughout is about 0.141 to about 2.1 pounds per minute.

The preheated mats pass to the coating section 14 where the mats are contacted with an anhydrous mixture of 70% to 95% by weight of stannous chloride and 5% to 30% by weight of stannous fluoride from raw material source 30. This contacting effects a coating of this mixture on the mats.

This contacting may occur in a number of different ways. For example, the  $\text{SnCl}_2/\text{SnF}_2$  mixture can be combined with nitrogen to form a vapor which is at a temperature of from about 25° C. to about 150° C. higher than the temperature of the mats in the coating section 14. As this vapor is brought into contact with the mats, the temperature differential between the mats and the vapor and the amount of the mixture in the vapor are such as to cause controlled amounts of  $\text{SnCl}_2$  and  $\text{SnF}_2$  to condense on and coat the mats.

Another approach is to apply the  $\text{SnCl}_2/\text{SnF}_2$  mixture in a molten form directly to the mats in an inert atmosphere. There are several alternatives for continu-

ously applying the molten mixture to the mats. Obtaining substantially uniform distribution of the mixture on the mats is a key objective. For example, the mats can be compressed between two rollers that are continuously coated with the molten mixture. Another option is to spray the molten mixture onto the mats. The fiber mats may also be dipped directly into the melt. The dipped fiber mats may be subjected to a compression roller step, a vertical lift step and/or a vacuum filtration step to remove excess molten mixture from the fiber mats.

An additional alternative is to apply the  $\text{SnCl}_2/\text{SnF}_2$  in an organic solvent. The solvent is then evaporated, leaving a substantially uniform coating of  $\text{SnCl}_2/\text{SnF}_2$  on the fiber mats. The solvent needs to be substantially non-reactive (at the conditions of the present process) and provide for substantial solubility of  $\text{SnCl}_2$  and  $\text{SnF}_2$ . For example, the dipping solution involved should preferably be at least about 0.1 molar in  $\text{SnCl}_2$ . Substantially anhydrous solvents comprising acetonitrile, ethyl acetate, dimethyl sulfoxide, propylene carbonate and mixtures thereof are suitable. Stannous fluoride is often less soluble in organic solvents than is stannous chloride. One approach to overcoming this relative insolubility of  $\text{SnF}_2$  is to introduce  $\text{SnF}_2$  onto the fiber mats after the fiber mats are dipped into the  $\text{SnCl}_2$  solution with organic solvent. Although the dopant may be introduced in the sintering section 18, it is preferred to incorporate the dopant in the coating section 14 or the equilibration section 16, more preferably the coating section 14.

Any part of process system 10 that is exposed to  $\text{SnCl}_2$  and/or  $\text{SnF}_2$  melt or vapor is preferably corrosion resistant, more preferably lined with inert refractory material.

In any event, the mats in the coating section 14 are at a temperature of up to about 375° C., and this section is operated at slightly less than atmospheric pressure. If the  $\text{SnCl}_2/\text{SnF}_2$  coating is applied as a molten melt between compression rollers, it is preferred that such compression rollers remain in contact with the fiber mats for about 0.1 to about 2 minutes, more preferably about 1 to about 2 minutes.

After the  $\text{SnCl}_2/\text{SnF}_2$  coating is applied to the fiber mats, the fiber mats are passed to the equilibration section 16. Here, the coated fiber mats are maintained, preferably at a higher temperature than in coating section 14, in a substantially inert atmosphere for a period of time, preferably up to about 10 minutes, to allow the coating to more uniformly distribute over the fibers. In addition, if the fluorine component is introduced onto the fiber mats separate from the stannous chloride, the time the coated fiber mats spend in the equilibration section 16 results in the dopant component becoming more uniformly dispersed or distributed throughout the stannous chloride coating. Further, it is preferred that any vapor and/or liquid which separate from the coated fiber mats in the equilibration section 16 be transferred back and used in the coating section 14. This preferred option, illustrated schematically in FIG. 1 by lines 32 (for the vapor) and 34 (for the liquid) increases the effective overall utilization of  $\text{SnCl}_2$  and  $\text{SnF}_2$  in the process so that losses of these components, as well as other materials such as solvents, are reduced.

The coated fiber mats are passed from the equilibration zone 16 into the sintering zone 18 where such fiber mats are contacted with an oxidizer, such as an oxygen-containing gas, from line 36. The oxidizer preferably

comprises a mixture of air and water vapor. This mixture, which preferably includes about 1% to about 50%, more preferably about 15% to about 35%, by weight of water, is contacted with the coated fiber mats at atmospheric pressure at a temperature of about 400° C. to about 550° C. for up to about 10 minutes. Such contacting results in converting the coating on the fiber mats to a fluorine doped tin dioxide coating. The fluorine doped tin oxide coated fiber mats product, which exits sintering section 18 via line 38, has useful electric conductivity properties. This product preferably has a doped tin oxide coating having a thickness in the range of about 0.5 microns to about 1 micron, and is particularly useful as a component in a lead-acid battery. Preferably, the product is substantially free of metals contamination which is detrimental to electrical conductivity.

The present process provides substantial benefits. For example, the product obtained has a fluorine doped tin oxide coating which has useful properties, e.g., outstanding electrical and/or morphological properties. This product may be employed in a lead-acid battery or in combination with a metallic catalyst to promote chemical reactions, e.g., chemical reductions, or alone or in combination with a metallic sensing component to provide sensors, e.g., gas sensors. High utilization of stannous chloride and fluorine components is achieved. In addition, high coating deposition and product throughput rates are obtained. Moreover, relatively mild conditions are employed. For example, temperatures within sintering section 18 can be significantly less than 600° C. The product obtained has excellent stability and durability.

In FIG. 2, an electromagnetic shielding element 50 is shown in use providing electromagnetic interference shielding for first component 52. That is, element 50 is in shielding relation to first component 52 relative to an electromagnetic interference source 54. In particular, element 50 is located between first component 52 and source 54. Element 50 and first component 52 may be parts of the same device, for example, element 50 being a housing for first component 52. Further, element 50 can act upon first component 52 in a shielding relation when first component 52 is a source of electromagnetic interference.

Referring to FIG. 4, element 50 is a flexible composite of a coated substrate 56 and a flexible, thermoplastic organic polymeric material 58. Coated substrate 56 is in the form of a randomly oriented, woven mat of C-glass fibers, a three dimensional substrate, and provides an electronically conductive path or network in element 50. As shown in FIG. 5, the individual coated fibers, illustrated by coated fiber 60, of coated substrate 56, are coated with a coating containing fluorine doped, electronically conductive tin oxide, illustrated by coating 62 on glass fiber 64.

In FIG. 3, an electrostatic dissipation element 70 is shown in use in contact with second component 72 to provide for dissipation of electrostatic energy. As is conventional, element 70 is grounded. Element 70 and second component 72 may be parts of the same article.

Referring to FIG. 6, element 70 is a flexible composite of coated substrate particles 74 oriented to provide an electrically conductive path or network in element 70, and a flexible, thermoplastic polymeric matrix material 76. Coated substrate particles 74 are three dimensional particles of various sizes and shapes and are coated with a coating containing fluorine-doped, electronically conductive tin oxide. In cross section, each of

these particles 74 looks much like individual fiber 60 in FIG. 5.

It should be noted that electromagnetic shielding element 50 can be structured as electrostatic dissipation element 70 is structured and vice versa.

The following non-limiting example illustrates certain aspects of the present invention.

#### EXAMPLE

10 A substrate made of C-glass was contacted with a molten mixture containing 30 mol % SnF<sub>2</sub> and 70 mol % SnCl<sub>2</sub>. This contacting occurred at 350° C. in an argon atmosphere at about atmospheric pressure and resulted in a coating containing SnCl<sub>2</sub> and SnF<sub>2</sub> being placed on the substrate.

15 This coated substrate was then heated to 375° C. and allowed to stand in an argon atmosphere at about atmospheric pressure for about 5 minutes. The coated substrate was then fired at 500° C. for 20 minutes using flowing, i.e., at the rate of one (1) liter per minute, water saturated air at about atmospheric pressure. This resulted in a substrate having a fluorine doped tin oxide coating with excellent electronic properties. For example, the volume resistivity of this material was determined to be  $7.5 \times 10^{-4}$  ohm-cm.

20 In the previously noted publication "Preparation of Thick Crystalline Films of Tin Oxide and Porous Glass Partially Filled with Tin Oxide and Porous Glass Partially Filled with Tin Oxide", an attempt to produce antimony doped tin oxide films on a 96% silica glass substrate involving stannous chloride oxidation at anhydrous conditions resulted in a material having a volume resistivity of  $1.5 \times 10^7$  ohm-cm.

25 The present methods and products, illustrated above, provide outstanding advantages. For example, the fluorine doped tin oxide coated substrate prepared in accordance with the present invention has improved, i.e., reduced, electronic resistivity, relative to substrates produced by prior methods.

30 35 40 While this invention has been described with respect to various specific examples and embodiments, it is to be understood that the invention is not limited thereto and that it can be variously practiced within the scope of the following claims.

45 What is claimed is:

1. An electrostatic dissipation/electromagnetic interference shielding element comprising an inorganic three dimensional substrate including external surfaces and shielded surfaces which are at least partially shielded by other portions of said substrate and having a dopant containing electronically conductive tin oxide coating on at least a portion of said external surfaces and said shielded surfaces, said coated substrate being adapted and structured to provide at least one of the following: electrostatic dissipation or electromagnetic interference shielding.

2. The element of claim 1 which further comprises a matrix material in contact with said coated substrate.

3. The element of claim 2 wherein said matrix material is an organic polymeric material.

4. The element of claim 3 wherein said coated substrate is in a form selected from the group consisting of spheres, flakes, irregularly shaped particles, fibers, fiber rovings, porous substrates and fiber mats.

5. The element of claim 3 wherein said coating further includes an effective amount of fluorine dopant.

6. The element of claim 3 wherein said coating has a thickness in the range of about 0.1 micron to 10 microns.

7. The element of claim 3 wherein said coated substrate is in a form selected from the group consisting of flakes and fibers.

8. The element of claim 7 wherein the ratio of the longest dimension to the shortest dimension of the substrate is in the range of from about 500:1 to about 10:1.

9. The element of claim 8 wherein the coated substrate is a flake and the longest length is less than about  $\frac{1}{8}$  inch.

10. The element of claim 8 wherein the organic polymeric material is a thermo plastic material and said coated substrate is in a form selected from the group consisting of flakes, irregularly shaped particles, and fibers.

11. The element of claim 3 wherein the organic polymeric material is a thermo plastic material and said coated substrate is in a form selected from the group consisting of flakes, irregularly shaped particles, and fibers.

12. The element of claim 1 wherein said coated substrate is produced in accordance with a process comprising:

contacting said substrate with a composition comprising a tin chloride-forming compound at conditions effective to form a liquidus tin chloride-containing coating on at least a portion of both said external surfaces and said shielded surfaces of said substrate; and

contacting said substrate having said tin chloride-containing coating thereon with an oxidizing agent at conditions effective to convert tin chloride to tin oxide.

13. The element of claim 1 wherein said coated substrate is in a form selected from the group consisting of spheres, flakes, irregularly shaped particles, fibers, fiber rovings, porous substrates and fiber mats.

14. The element of claim 1 wherein said coating further includes an effective amount of fluorine dopant.

15. The element of claim 14 which further comprises a cured or uncured polymer based carrier and the coated substrate is in a form selected from the group consisting of spheres, flakes, irregularly shaped particles, and fibers.

16. The element of claim 1 wherein said coating has a thickness in the range of about 0.1 micron to 10 microns.

17. The element of claim 1 which further comprises a cured or uncured polymer based carrier and the coated substrate is in a form selected from the group consisting of spheres, flakes, irregularly shaped particles, and fibers.

18. The element of claim 1 which further comprises a cured or uncured polymer based carrier and the coated substrate is in a form selected from the group consisting of spheres, flakes, irregularly shaped particles, and fibers, the longest dimension is less than about  $\frac{1}{8}$  inch and the ratio of the longest dimension to the shortest dimension is in the range of about 500:1 to about 10:1.

19. A flexible electrostatic dissipation/electromagnetic shielding element comprising a flexible matrix

material in contact with an inorganic three dimensional substrate including external surfaces and shielded surfaces which are at least partially shielded by other portions of said substrate and having a dopant containing electronically conductive tin oxide coating on at least a portion of said external surfaces and said shielded surfaces said coated substrate being adapted and structured to provide at least one of the following: electrostatic dissipation or electromagnetic interference shielding.

20. The element of claim 19 wherein said matrix material is an organic polymeric material.

21. The element of claim 20 wherein said coated substrate is in a form selected from the group consisting of spheres, flakes, irregularly shaped particles, fibers, fiber rovings, porous substrates, and fiber mats.

22. The element of claim 20 wherein said coating further includes an effective amount of fluorine dopant.

23. The element of claim 20 wherein said coating has a thickness in the range of about 0.1 micron to about 10 microns.

24. The element of claim 20 wherein said coated substrate is in a form selected from the group consisting of flakes and fibers.

25. The element of claim 24 wherein the ratio of the longest dimension to the shortest dimension of the substrate is in the range of from about 500:1 to about 10:1.

26. The element of claim 25 wherein the organic polymeric material is a thermo plastic material and said coated substrate is in a form selected from the group consisting of flakes, irregularly shaped particles, and fibers.

27. The element of claim 20 wherein the organic polymeric material is a thermo plastic material and said coated substrate is in a form selected from the group consisting of flakes, irregularly shaped particles, and fibers.

28. The element of claim 19 wherein coated substrate is produced in accordance with a process comprising: contacting said substrate with a composition comprising a tin chloride-forming compound at conditions effective to form a liquidus tin chloride-containing coating on at least a portion of both said external surfaces and said shielded surfaces of said substrate; and

contacting said substrate having said tin chloride-containing coating thereon with an oxidizing agent at conditions effective to convert tin chloride to tin oxide.

29. The element of claim 19 wherein said coated substrate is in a form selected from the group consisting of spheres, flakes, irregularly shaped particles, fibers, fiber rovings, porous substrates and fiber mats.

30. The element of claim 19 wherein said coating further includes an effective amount of fluorine dopant.

31. The element of claim 19 wherein said coating has a thickness in the range of about 0.1 micron to 10 microns.

\* \* \* \* \*